

Patented Dec. 7, 1926.

## UNITED STATES PATENT OFFICE.

RICHARD WALTER, OF NUREMBERG, GERMANY.

## PROCESS OF APPLYING A METALLIC LAYER TO ANOTHER METAL.

No Drawing.

Application filed October 31, 1925. Serial No. 66,070.

My invention pertains to a process of applying a metallic layer of desired thickness upon another metal so that the contacting surfaces of both metals completely adhere to each other, without possibility of separation. The invention is especially adapted for use when it is intended to apply a layer of metal like nickel or chromium or alloys of the iron or chromium group upon a common or base metal like iron. A distinguishing feature of my invention is the accomplishment of the union of the two distinct metals by use of the one metal in its molten state while a more common metal retains its solid form, and while preventing oxidation, so as to effect a lasting union and preserve the quality of the applied layer of metal.

Processes have been known, according to which two metals were joined in similar manner, but I have discovered that the methods heretofore practiced involved two serious shortcomings which considerably lowered the quality of the product. According to such defective methods, the base upon which the layer of metal should be applied while in its molten state, must be preheated to the maximum feasible temperature in order that the molten metal becomes welded thereto when it impinges. The necessarily high preheating results in the underlying metal becoming more or less oxidized by reason of the oxygen in the air and in consequence frustrates a reliable union of it with the molten metal. If such oxidation occurs, the two metals will not weld over their entire contacting surfaces, but are only sporadically stuck together and will therefore again separate during use. That is the more likely often to occur when two metal elements which are so attached later become subjected to an operation like rolling, tension or cutting.

I have moreover discovered that the quality of the fluid-applied metal suffered appreciably during the practice of previously known methods owing to its exposure to atmospheric oxygen while poured or deposited dropwise upon the base and thereby became more or less oxidized or impregnated with gases of oxygen content. This is especially apt to occur when the molten metal used does not belong to the iron group, but to that of manganese, cobalt, nickel, also to constituents of the chromium group such as chromium, tungsten, molyb-

dium and uranium which have a high affinity for oxygen.

Accordingly, the successfully attained objects of my invention have been to prevent oxidation of the underlying metal which it is required to preheat as well as to prevent absorption of oxygen by the gravitationally applied molten metal. I achieve the desired ends by directing the jet of reducing gas flame against that portion of the surface of the underlying metal base upon which the molten metal is to be poured or dropped. The gas may be hydrogen, carbon monoxide or in some instances acetylene or other carbohydrates, and its application quite prevents oxidation, so that I can carry the preheating of the lower metallic layer to a stage in which its upper surface commences to melt, whereby an absolute fusion with the molten metal is assured.

The second operation of my method consists in surrounding the applied molten metal with a reducing-gas stream of the character above stated from the time of commencement of its liquefaction and further in enveloping the stream or drops of the molten metal with the reducing jet while being deposited upon the base metal.

My process of absolutely preventing the access of air and of obtaining the high degree of localized heating of the base permits me to realize a product in which the two metallic layers are homogeneously alloyed over the entire area of their contacting surfaces and in which the applied layer of metal preserves its high quality. If required, the products of my method may be subjected to any additional manufacturing process without danger of separation of the two metal layers. In certain cases, for example when the form of the work piece allows, the reducing agency may be simultaneously utilized to preheat the base or melt the other metal or to perform both operations in unison.

I claim:

1. The step in the process of depositing a metal layer upon another metal by pouring molten metal upon another highly heated metal which consists in effecting the preheating of the metal constituting the receiving base by continuous application of a reducing gas stream over that portion of the surface of said base which is to be covered by the molten metal whereby to preclude oxidation.

2. The process as specified in claim 1, in which the preheating of the metal-base progresses under the complete protection of the reducing gases until all of its surface which is to be covered with molten metal just reaches fusion temperature while preventing oxidation by exclusion of air.
3. The process according to claim 1, in which molten metal is enveloped in a stream of reducing gas to accomplish its liquefaction and thereafter likewise enveloped by said reducing gas stream during its application to the base metal.
4. The process according to claim 1, in which the applied molten metal is enveloped in a stream of reducing gas both during its liquefaction and during its pouring or dropping.
5. The process as specified in claim 1, in which the reduction gases are utilized simultaneously to heat the base layer of metal and to liquefy the other metal.
6. The process of applying a metal layer upon another metal by depositing molten metal upon another highly heated metal which consists in effecting the melting of the metal to be deposited by enveloping it in a reducing gas stream during a gravitational deposition thereof.

Signed by me, this 28th day of October, 1925.

RICHARD WALTER.